

Patented Mar. 15, 1927.

1,620,715

# UNITED STATES PATENT OFFICE.

FRANK H. BERGEIM, OF WOODBURY, NEW JERSEY, ASSIGNOR TO E. I. DU PONT DE NEMOURS & COMPANY, OF WILMINGTON, DELAWARE, A CORPORATION OF DELAWARE.

## EXPLOSIVE COMPOSITION.

No Drawing. Original application filed June 18, 1926, Serial No. 116,977. Divided and this application filed September 9, 1926. Serial No. 134,583.

My invention relates particularly to compositions containing an explosive having one or more triazo groups and one or more nitrate groups, but it has relation especially to compositions containing an explosive in which a hydrocarbon has attached thereto one or more of each of said groups.

This application is a division of my co-pending application upon triazo nitrate explosives and process of producing the same, Serial No. 116,977, filed June 18, 1926.

The object of my invention is to provide an explosive composition containing a new type of explosive of the above character combining in part the explosive groupings of two well-known high explosives, lead azide and nitroglycerine. The object of my invention is particularly to provide compositions containing an explosive of this type in which one or more triazo

different kinds of alcohols may be so treated in order to obtain the corresponding triazo nitrates. In general, it will be found, however, that the shorter the hydrocarbon chain and the smaller the number of carbon atoms in relation to the triazo and nitrate groups, the greater the sensitiveness of the explosive. Also, it will be understood that for this purpose any of the triazo alcohols used for nitration in this way may be prepared from the corresponding halo-hydribs by any of the known methods of replacing the halogen by the triazo group, as, for example, as described by Forster and Fierz. in J. Chem. Soc. (1908) 93-1865, relating to the treatment of ethylene chlorohydrin with sodium azide.

In carrying out my invention, the explosives for use in compositions made in accordance with my invention may be made in any suitable way but, for example, in the preparation of triazo-ethanol-nitrate I may add one part by weight of triazo ethanol to two parts by weight of mixed acids comprising approximately 40% nitric acid and 60% sulphuric acid, either in the absence of water or with not more than 10% water present, the temperature being kept between 0° and 5° C. The triazo ethanol nitrate formed collects on the surface of the waste acid and may be drawn off therefrom and washed repeatedly until neutral, with the aid of a weakly alkaline water solution such as a 5% solution of sodium carbonate in water. The triazo-ethanol-nitrate obtained is a colorless, neutral mobile oil having a specific gravity of about 1.3. It has considerably greater sensitiveness to mechanical shock than nitroglycerine, as shown by the drop weight method. Furthermore, it has a somewhat greater strength than nitroglycerine, as shown by the ballistic mortar test.

The triazo-ethanol-nitrate as prepared above is a high explosive in itself and may be used in any desired type of explosive composition, for example, in combination with the usual ingredients of dynamite to make a dynamite of great strength and sensitiveness. It may be used in a dynamite comprising nitroglycerine or its equivalent, as, for example, mixtures of nitroglycerine with tetratinitro diglycerine, nitro sugars or



groups, as well as one or more nitrate ( $-\text{ONO}_2$ ) groups are attached to a hydrocarbon. The simplest example of such an explosive is triazo-ethanol-nitrate,



an explosive having greater strength and sensitiveness than nitroglycerine.

While my invention is capable of being carried out in many different ways I shall describe only certain ways of carrying out the same hereinafter.

The triazo nitrates as above referred to may be made in any desired way but, for example, they may be made by treating a triazo alcohol with mixed acids. For instance, if the triazo alcohol to be treated is triazo-ethanol  $\text{N}_3\text{CH}_2\text{CH}_2\text{OH}$ , the explosive obtained therefrom will be triazo-ethanol-nitrate  $\text{N}_3\text{CH}_2\text{CH}_2\text{ONO}_2$ , the structural formula of which is



Again, in case a triazo polyhydric alcohol, as, for example, a triazo glycol, is nitrated, triazo propylene glycol dinitrate



is obtained. In this way many and various

nitroglycol. The following composition may be cited as a specific example of a dynamite in which the new explosive may be used:

|                          | Parts by weight. |
|--------------------------|------------------|
| 5 Triazo-ethanol-nitrate | 15               |
| Glycerine trinitrate     | 15               |
| Sodium nitrate           | 57               |
| Wood meal                | 12               |
| 10 Chalk                 | 1                |

It is also to be understood that any of the triazo nitrate explosives may be used in accordance with my invention as a substitute 15 for nitroglycerine in any of the explosive compositions in which the latter is used, as, for example, in any of the known dynamite compositions. For example, such explosives 20 may be used with nitrocellulose to form gelatinized explosives.

Furthermore, instead of the sodium nitrate, or in addition thereto, I may use various other oxidizing salts, as, for example, ammonium nitrate, ammonium perchlorate 25 or potassium nitrate. Also, it will be understood that the various known carbonaceous combustibles for use in explosives may be used in connection therewith instead of and together with the wood meal. Also, 30 other mineral fillers may be used instead of or together with the chalk hereinabove referred to.

It is to be understood, however, that in all the above compositions the proportions 35 may vary widely as to each and all of the ingredients, according to the particular uses to which the explosive is to be applied.

While I have described my invention above in detail I wish it to be understood 40 that many changes may be made therein without departing from the spirit of the same.

I claim:

1. An explosive composition containing a 45 compound having therein a triazo group and a nitrate group.
2. An explosive composition containing a compound comprising a hydrocarbon ester having therein a triazo group and a nitrate group.
3. An explosive composition containing a compound comprising an aliphatic hydrocarbon ester having therein a triazo group and a nitrate group.
4. An explosive composition containing a compound comprising an aliphatic hydrocarbon ester having therein a triazo group and a nitrate group, said groups being each attached to different carbon atoms therein.
5. A dynamite having therein an explosive compound containing a triazo group and a nitrate group.
6. A dynamite having therein an explosive compound comprising a hydrocarbon ester containing a triazo group and a nitrate group.

sive compound comprising a hydrocarbon ester containing a triazo group and a nitrate group.

7. A dynamite having therein an explosive compound comprising an aliphatic hydrocarbon ester containing a triazo group and a nitrate group.

8. A dynamite having therein an explosive compound comprising an aliphatic hydrocarbon ester containing a triazo group and a nitrate group, said groups being each attached to different carbon atoms therein.

9. A dynamite having therein an explosive compound containing a triazo group and a nitrate group, and an absorbent.

10. A dynamite having therein an explosive compound containing a triazo group and a nitrate group, an absorbent, and an oxidizing agent.

11. A dynamite having therein an explosive compound containing a triazo group and a nitrate group, wood meal, and sodium nitrate.

12. A dynamite having therein an explosive compound comprising a hydrocarbon ester containing a triazo group and a nitrate group, and an absorbent.

13. A dynamite having therein an explosive compound comprising a hydrocarbon ester containing a triazo group and a nitrate group, an absorbent, and an oxidizing agent.

14. A dynamite having therein an explosive compound comprising a hydrocarbon ester containing a triazo group and a nitrate group, wood meal, and sodium nitrate.

15. A dynamite having therein an explosive compound comprising an aliphatic hydrocarbon ester containing a triazo group and a nitrate group, and an absorbent.

16. A dynamite having therein an explosive compound comprising an aliphatic hydrocarbon ester containing a triazo group and a nitrate group, an absorbent, and an oxidizing agent.

17. A dynamite having therein an explosive compound comprising an aliphatic hydrocarbon ester containing a triazo group and a nitrate group, wood meal, and sodium nitrate.

18. A dynamite having therein an explosive compound comprising triazo-ethanol-nitrate, and an absorbent.

19. A dynamite having therein an explosive compound comprising triazo-ethanol-nitrate, an absorbent, and an oxidizing agent.

20. A dynamite having therein an explosive compound comprising triazo-ethanol-nitrate, wood meal, and sodium nitrate.

In testimony that I claim the foregoing, I have hereunto set my hand this 2nd day of September, 1926.

FRANK H. BERGEIM.